



US007763213B2

(12) **United States Patent**  
**Miksic et al.**

(10) **Patent No.:** **US 7,763,213 B2**  
(45) **Date of Patent:** **Jul. 27, 2010**

(54) **VOLATILE CORROSION INHIBITOR  
PACKAGES**

(75) Inventors: **Boris A. Miksic**, North Oaks, MN (US); **Cliff Cracauer**, Oakdale, MN (US); **Brian Wuertz**, Fridley, MN (US); **Scott Bolton**, Austin, TX (US); **Barry Haygood**, Austin, TX (US); **Grant McEwan**, Austin, TX (US)

(73) Assignees: **Freescale Semiconductor, Inc.**, Austin, TX (US); **Cortec Corporation**, St. Paul, MN (US)

(\*) Notice: Subject to any disclaimer, the term of this patent is extended or adjusted under 35 U.S.C. 154(b) by 1160 days.

(21) Appl. No.: **11/314,220**

(22) Filed: **Dec. 21, 2005**

(65) **Prior Publication Data**

US 2007/0138031 A1 Jun. 21, 2007

(51) **Int. Cl.**

*A61L 9/00* (2006.01)  
*A62B 7/08* (2006.01)  
*B65D 81/24* (2006.01)  
*C09K 3/00* (2006.01)  
*A21D 10/02* (2006.01)  
*B32B 3/12* (2006.01)  
*B32B 27/00* (2006.01)  
*B32B 5/18* (2006.01)  
*B32B 27/04* (2006.01)  
*B32B 27/12* (2006.01)  
*A01M 13/00* (2006.01)  
*B65B 41/18* (2006.01)

(52) **U.S. Cl.** **422/123; 422/1; 422/5; 422/28; 422/305; 206/205; 252/194; 426/118; 428/425.5; 428/424.7; 428/118; 442/118; 442/76; 442/131; 442/286; 442/268; 43/124; 43/125; 53/425; 53/170; 53/562; 53/285; 53/381.1; 53/393; 53/452**

(58) **Field of Classification Search** ..... 442/1, 442/5, 28, 123, 305, 118, 76, 131, 286, 268; 206/205; 252/194; 426/118; 428/425.5, 428/424.7, 118; 422/1, 5, 28, 123, 305; 43/124-125; 53/425, 170, 562, 285, 381.1, 393, 452  
See application file for complete search history.

(56) **References Cited**

**U.S. PATENT DOCUMENTS**

4,597,218 A \* 7/1986 Friemel et al. ..... 43/131  
4,973,448 A 11/1990 Carlson et al. .....  
5,139,700 A 8/1992 Miksic et al. .....  
5,209,869 A 5/1993 Miksic et al. .....  
5,332,525 A 7/1994 Miksic et al. .....  
5,378,428 A \* 1/1995 Inoue et al. ..... 422/9  
5,422,187 A \* 6/1995 Miksic et al. ..... 428/545

(Continued)

**OTHER PUBLICATIONS**

International Search report for corresponding PCT Application No. PCT/US06/62292 dated Sep. 28, 2007.

*Primary Examiner*—Jill Warden  
*Assistant Examiner*—Monzer R Chorbaji

(57) **ABSTRACT**

A package for enclosing volatile corrosion inhibiting materials includes a first enclosure barrier being fabricated from one or more gas-impermeable materials and defining a first enclosed space. The package further includes a substrate having one or more volatile corrosion inhibitor materials disposed thereon, with the substrate being disposed within the first enclosed space. In some embodiments, a second enclosure barrier being fabricated from a gas-permeable, solid particle-impermeable material is disposed in the first enclosed space, and defines a second enclosed space inside of the first enclosed space. In such embodiments, the substrate is preferably disposed within the second enclosed space.

**26 Claims, 4 Drawing Sheets**



U.S. PATENT DOCUMENTS

5,545,289 A 8/1996 Chen et al.  
6,028,160 A 2/2000 Chandler et al.  
6,080,334 A 6/2000 Heimann et al.

6,146,730 A 11/2000 Lewis et al.  
6,551,552 B1 4/2003 Lyublinski et al.  
6,617,415 B1 9/2003 Miksic et al.

\* cited by examiner





Fig. -4





*Fig.-5*

**1**  
**VOLATILE CORROSION INHIBITOR  
PACKAGES**

FIELD OF THE INVENTION

The present invention relates to packages enclosing volatile corrosion inhibitor-containing materials generally, and more particularly to packaging incorporating an outer gas-impermeable barrier and an inner gas-permeable, solid particle-impermeable barrier within which a volatile corrosion inhibitor-containing substrate is contained.

BACKGROUND OF THE INVENTION

Volatile corrosion inhibitor materials, such as vapor phase corrosion inhibitors, are widely utilized as species impregnated within or otherwise disposed upon various substrates. The volatile corrosion inhibitor (VCI) materials emit vapor phase corrosion inhibitors over time, even at ambient conditions, such that by placing the VCI-containing substrate at a location adjacent to corrosion-susceptible materials, the vapor phase corrosion inhibitors operably act to protect such materials from corrosion.

In some embodiments of the prior art, volatile corrosion inhibitor materials have been incorporated into films for use as barrier layers to enclose corrosion-susceptible items. In such embodiments, vapor phase corrosion inhibitors are released from the barrier film to engage with the enclosed item so as to protect the item from corrosion.

In other embodiments of the prior art, volatile corrosion inhibitor materials have been incorporated with a substrate to form a corrosion inhibiting product that may be placed adjacent to corrosion-susceptible items. A wide variety of substrates in a wide variety of configurations are useful in releasably containing the volatile corrosion inhibitor materials, with such substrates being fabricated from, for example, non-woven fabrics, paper, polymeric films, and foam materials, such as open cell urethane foams. In certain applications, adhesives may be applied to a surface of the substrate, such that the corrosion inhibiting product may be adhesively affixed to a location adjacent to the targeted corrosion-susceptible items.

It has been found that such corrosion inhibiting products may be disposed within a permeable enclosure that allows the vapor phase corrosion inhibitor to be emitted out from within the enclosure to protect adjacent corrosion-susceptible items. An example permeable enclosure for volatile corrosion inhibitor materials is described in U.S. Pat. No. 5,422,187, which is incorporated herein by reference. The permeable enclosure barrier described in U.S. Pat. No. 5,422,187 allows vapors to pass therethrough but prevents emission of solid particles out from the enclosure.

A particular application for corrosion inhibitor products contained within a gas-permeable enclosure is in the fabrication of semiconductors and related electronic components. Such components are typically manufactured in "clean room" environments so as to prevent contamination during the manufacturing process. In addition to attempting to prevent particle contamination of such electronic components, manufacturers have also taken steps to minimize exposure to moisture and other airborne chemical contaminants, which can partially corrode delicate metal elements in the electronic devices. One measure commonly taken is to limit the time of exposure to the clean room environment between processing steps which expose metal surfaces of the electronic device. These queue times in conjunction with ambient moisture

**2**

controls are used to successfully process semiconductor devices without incurring corrosion of metallic features.

It has been found that volatile corrosion inhibitor products can assist in preventing corrosion damage to such electronic components by placing the corrosion inhibiting products in proximity to the electronic components to thereby expose such components to vapor phase corrosion inhibitors. To eliminate the risk of particle contamination of the electronic components, from, for example, degradation of the corrosion inhibitor product or emission of solid volatile corrosion inhibitors, the corrosion inhibitor products are preferably enclosed within a gas-permeable, solid particle-impermeable barrier.

In researching the effectiveness of currently available gas-permeable barrier enclosed corrosion inhibitor products, Applicants have determined that a relatively high concentration of vapor phase corrosion inhibitors present in a treatment zone is desired for insuring corrosion protection of the electronic components stored therein. However, due to the volatile nature of the corrosion inhibitor materials in the corrosion inhibitor products, the effectiveness of such corrosion inhibitor products decreases over time when exposed to ambient conditions as a result of vapor pressure equilibration effects. In the course of experimentation and testing, it has now been discovered that corrosion inhibitor products disposed in gas-permeable barriers alone have the tendency to lose effectiveness over time.

In addition, it has been found that the release rate of vapor phase corrosion inhibitors from the corrosion inhibiting products is limited by the total surface area of the supporting substrate that is capable of emitting vapor phase corrosion inhibitors to the ambient surroundings.

Accordingly, it is a principal object of the present invention to provide a volatile corrosion inhibitor package that incorporates a gas-impermeable outer enclosure barrier that maintains a desired elevated corrosion inhibitor vapor pressure adjacent to the corrosion inhibitor product.

It is a further object of the present invention to provide a volatile corrosion inhibitor package that incorporates an outer gas-impermeable barrier layer and a gas-permeable, solid particle-impermeable inner barrier layer within which a corrosion inhibitor product is disposed until it is ready for use.

It is a still further object of the present invention to provide a corrosion inhibitor product having an enhanced emission surface area for accelerating release of vapor

BRIEF DESCRIPTION OF THE DRAWINGS

FIG. 1 is a cross-sectional side view of a corrosion inhibitor package of the present invention;

FIG. 2 is a cross-sectional side view of a corrosion inhibitor package of the present invention;

FIG. 3 is a cross-sectional side view of a corrosion inhibitor package of the present invention; and

FIG. 4 is a cross-sectional side view of a corrosion inhibitor package of the present invention.

FIG. 5 is a graph of time-to-flight surface ion mass spectroscopy (TOF-SIMS) on copper wafers.

DETAILED DESCRIPTION OF THE PREFERRED  
EMBODIMENTS

The objects and advantages enumerated above together with other objects, features, and advances represented by the present invention will now be presented in terms of detailed embodiments described with reference to the attached drawing figures which are intended to be representative of various

possible configurations of the invention. Other embodiments and aspects of the invention are recognized as being within the grasp of those having ordinary skill in the art.

With reference now to the drawing figures, and first to FIG. 1, a vapor phase corrosion inhibiting package 10 includes a first enclosure barrier 12 defining a first enclosed space 14, a second enclosure barrier 16 disposed in first enclosed space 14, and itself defining a second enclosed space 18 therewithin. Corrosion inhibiting package 10 preferably further includes a substrate 22 disposed within second enclosed space 18, with substrate 22 including volatile corrosion inhibitor materials disposed thereon and therein.

First enclosure barrier 12 is preferably fabricated from a gas-impermeable material that both prevents moisture or other vapor phase materials from penetrating into first enclosed space 14, and prevents vapor phase corrosion inhibitor materials emitted from substrate 22 from passing therethrough. In preferred embodiments, therefore, first enclosure barrier 12 is fabricated from a gas-impermeable material such as a metallized film. Such metallized films may also include metallized film laminates. A particular example of a material useful in first enclosure barrier 12 is polyethylene terephthalate film containing a vapor deposited film or layer of metallic aluminum. Such films are commercially available and are commonly designated as "metallized" films.

Preferably, first enclosure barrier 12 is formed by sealing together two distinct film layers 12A, 12B at perimeter sealing edges 11A, 11B. Conventional sealing mechanisms may be employed for obtaining a gas-tight seal at the perimeter seal edge 11A, 11B, with such sealing techniques including, for example, heat-sealing, ultra-sonic sealing, and the like. Preferably, second enclosure barrier 16 and substrate 22 are placed upon a respective inner surface of one or both of first and second film layers 12A, 12B prior to the sealing process.

In other embodiments, however, first enclosure barrier 12 may be formed of a single film layer operably secured and sealed to a base layer, with both layers being gas-impermeable materials. By way of example, first metallized film layer 12A may be secured to an aluminum plate (not shown) for sealably enclosing second enclosure barrier 16 and substrate 22. While the present invention contemplates a variety of materials and methods for obtaining first enclosure barrier 12, it is a principle object of the invention to obtain a gas-impermeable barrier within which second enclosure barrier 16 and substrate 22 are operably disposed. Moreover, first enclosure barrier 12 is preferably configured so as to be openable by the user, such that the user may operably position corrosion inhibitor product 6, which is the combination of second enclosure barrier 16 and substrate 22, at desired locations for effecting a vapor phase corrosion inhibition characteristic. Specifically, first enclosure barrier 12 is preferably configured to only temporarily contain corrosion inhibitor product 6, such that when the user desires the release of vapor phase corrosion inhibitors from corrosion inhibitor product 6, such user may operably remove corrosion inhibitor product 6 from within first enclosure barrier 12.

Accordingly, first enclosure barrier 12 acts to maintain an environment in first enclosed space 14 having an elevated vapor pressure for the volatile corrosion inhibitors disposed on and in substrate 22. In such an environment, an equilibrated vapor pressure between an outer surface 24 of substrate 22 and first and second enclosed space 14, 18 is quickly achieved. The rapid equilibration of vapor pressures results in a retention and equilibrium by substrate 22 of the volatile corrosion inhibitor material originally disposed therat. Such a characteristic leads to a relatively "fresh" corrosion inhibitor product 6 at the ultimate point of use, which could be

several days or months subsequent to original product manufacture. In other words, corrosion inhibitor product 6 is prevented from emitting a substantial portion of the volatile corrosion inhibitor materials originally incorporated into substrate 22 prior to the time at which the user removes corrosion inhibitor product 6 from within first enclosed space 14.

Second enclosure barrier 16 is preferably a gas-permeable, but solid particle-impermeable material that provides for the 10 emission of vapor phase corrosion inhibitors therethrough. However, the material making up second enclosure barrier 16 prevents solid particles from passing therethrough, thereby preventing solid particle contamination of the environment external to second enclosure barrier 16.

15 Although a variety of clean-room approved, gas-permeable fabrics are envisioned for use in the second enclosure barrier 16 of the present invention, exemplary preferred materials include Tyvek® 1059 which is available from E.I. du Pont de Nemours and Company under the "Tyvek®" class of 20 materials, and those available from W.L. Gore, Inc. under the trade name "Goretex®". In a further aspect of the invention, use of the above-cited materials provides mono-direction emissivity, such that vapors are only allowed to pass through second enclosure barrier 16 from within second enclosed 25 space 18. As such, water vapor and other vapor-borne contaminants are prevented from entering second enclosed space 18. Such a characteristic is important to the longevity of the present invention, in that certain vapor substances have been found to degrade substrate 22 and otherwise limit the effectiveness of corrosion inhibitor product 6.

30 As shown in FIG. 1, second enclosure barrier 16 is preferably formed of two distinct film layers 16A, 16B, and sealed together through conventional sealing techniques at perimeter sealing edges 15A, 15B. Second enclosure barrier 16 35 may be formed of homogeneous or heterogeneous films. In one embodiment, for example, first film layer 16A may be fabricated from a 0.125-0.175 mm caliper thickness Tyvek® fabric, while second film layer 16B may be fabricated from different materials, such as polyethylene having a caliper 40 thickness of about 0.05-10 mm. Such a heterogeneous configuration for second enclosure barrier 16 reduces material costs in that Tyvek® material is substantially more expensive than more commonly utilized polymeric films, and enhances the overall durability of corrosion inhibitor product 6. Such 45 durability may be further enhanced by creating second film layer 16B of a relatively durable polymeric material such as polyethylene. In such an embodiment, only a portion of second enclosure barrier 16 is fabricated from a relatively thin layer of e.g. Tyvek®.

50 Of course, since at least a portion of second enclosure barrier 16 is fabricated from a gas-permeable material, first and second enclosed spaces 14, 18 are in at least gaseous communication with one another. As a result, the vapor pressures of the respective volatile corrosion inhibitor material is 55 in operable equilibrium with one another. By minimizing the volume of first enclosed space 14 external to second enclosure barrier 16, reduction in vapor phase corrosion inhibitor potential, as measured from an original "charge" of material at manufacture, is minimized.

60 As indicated above, substrate 22 is preferably disposed in second enclosed space 18, and may be either freely disposed therein, or may alternatively be adhered to a respective inner surface of second enclosure barrier 16. Although substrate 22 65 may be any of a variety of materials and configurations useful in at least temporarily retaining volatile corrosion inhibitor material thereat, a particularly preferred material for use in corrosion inhibitor product 6 of the present invention is an

open cell isocyanate-derived or urethane foam. Materials and methods for impregnating or otherwise incorporating volatile corrosion inhibitor material within substrate 22 are described in, for example, U.S. Pat. No. 5,422,187. As described therein, open cell foam substrate 22 is preferably impregnated with volatile corrosion inhibitor material by immersing substrate 22 in a liquid solution containing the volatile corrosion inhibitor material. Subsequent evaporation of the solvent from substrate 22 yields an impregnated foam product. Various ratios of ingredients may be impregnated in substrate 22, with certain volatile corrosion inhibitor material being useful for the particular corrosion-susceptible materials in need of corrosion protection.

Other methods and materials for obtaining substrate 22, however, are contemplated by the present invention. For example, a porous paper or non-woven fabric may be impregnated with volatile corrosion inhibitor material in solid or liquid form.

In certain applications of the present invention, such as in the corrosion protection semiconductor wafers, it has been found that substrate 22 is most useful in a configuration forming a planar surface that is placed within close proximity to the surface of exposed metal features of the semiconductor wafers. Preferably, such proximity is between about 2 and 10 mm. Such a wafer to substrate orientation may be achieved within an enclosed environment such as a lot box or other container to hold a plurality of semiconductor wafers in the presence of one or more corrosion inhibitor-containing substrates for a defined period of time to deposit a protective corrosion inhibitor layer upon the semiconductor wafers.

In preferred embodiments of the present invention, substrate 22 contains between about 35 and 60% by weight volatile corrosion inhibitor material. In embodiments utilizing open cell foam as the material for substrate 22, the volatile corrosion inhibitor materials are preferably present at between 40% and 65% by volume of the total substrate volume, depending upon the density of the foam construction. Such concentrations of volatile corrosion inhibitor material have been found to provide a desired level of corrosion protection upon adjacent corrosion-susceptible items, and particularly for electronic components disposed in a conventionally arranged lot box.

As shown in FIG. 2, a further embodiment of the present invention is provided wherein substrate 23 of corrosion inhibiting package 20 is in the form of ground pieces of substrate 22. As such, substrate 23 is in the form of a plurality of distinct pieces having a mean diameter of between about 0.25 and about 0.5 mm. Most preferably, substrate 23 is in the form of a plurality of distinct open cell foam pieces, with the average loading of volatile corrosion inhibitor material in the substrate pieces 23 being between about 35 and 60% by weight.

As described above, one aspect of the present invention is in the rapid disbursement of vapor phase corrosion inhibitor once corrosion inhibitor package 6 is removed from first enclosure barrier 12. The embodiment of substrate 23 illustrated in FIG. 2 enables such a rapid dispersion by significantly increasing the surface area of loaded substrate 23 exposed to the ambient environment once corrosion inhibitor product 6 is removed from first enclosure barrier 12. The embodiment of substrate 23 in the form of a plurality of distinct foam pieces provides several magnitudes greater total VCI release surface area.

An additional embodiment of the present invention is illustrated in FIG. 3, wherein substrate 22 is disposed within first enclosed space 14 defined by first enclosure barrier 12. Thus, vapor phase corrosion inhibiting package 30 enables the con-

tainment of volatile corrosion inhibitors within enclosed space 14 without the utilization of second enclosure barrier 16.

A further embodiment of the corrosion inhibiting package of the present invention is illustrated in FIG. 4, wherein package 40 includes a structure 42 having a first open end 44 defining a chamber 46 in communication with first open end 44. Structure 42 is preferably fabricated from a gas-impermeable material such as polyethylene. In preferred embodiments, structure 42 has a wall thickness sufficiently large so as to render structure 42 self-supporting in a pre-defined configuration. As such, the wall thickness of structure 42 is preferably between about 0.25 and 10 mm, and more preferably between about 0.5 and 2 mm.

A first barrier layer 56 is preferably disposed at and encloses first open end 44 of structure 42. In preferred embodiments, first barrier layer 56 is secured to annular flange 43 of structure 42 through heat sealing, ultrasonic bonding, adhesive bonding, or other conventional bonding techniques. First barrier layer 56 is preferably a gas-permeable, solid particle-impermeable material, as described above.

Package 40 preferably further includes a second barrier layer 52 superimposed over first barrier layer 56, and secured to structure 42, such as at annular flange 43 of structure 42. Second barrier layer 52 is preferably secured to structure 42 through well known techniques, such as those described above. Second barrier layer 52 is preferably fabricated from a gas-impermeable material and is preferably positioned at package 40 so as to enclose first barrier layer 56 within a first enclosure defined by structure 42 and second barrier layer 52. Such an enclosure is therefore gas-impermeable so as to rapidly equilibrate the vapor pressure of corrosion inhibiting materials, as between chamber 46 and substrate 22. Such an enclosure thereby inhibits the degradation of corrosion inhibiting effectiveness over time of substrate 22.

In accordance with a preferred embodiment of the present invention, package 40 of the present invention may be utilized by breaching second barrier layer 52 through penetration thereof or some other fashion in order to render chamber 44 in gas communication with the ambient environment external to package 40. Such breaching may be accomplished by, for example, creating one or more apertures in second barrier layer 52 with a piercing object, removing portions of second barrier layer 52 sufficient to enable vapor transfer between chamber 46 and the ambient environment external to structure 42, and/or removal of second barrier layer 52 substantially in its entirety. Once such exposure has been effected, package 40 is preferably placed in proximity to a corrosion-susceptible material, such as metal surfaces of semiconductor devices. A proximity of between about 0.5 and 30 cm provides a preferred degree of vapor phase corrosion inhibitor deposition upon such corrosion-susceptible materials for protection thereof from corrosion effects. It is also contemplated by the present invention that package 40, for example, may be provided without first barrier layer 56, such that only second barrier layer 52 seals chamber 46 until selectively breached by the user.

Specific embodiments of the present invention are further illustrated by the following examples. Such examples, how-

ever, should not be construed as being limiting to the scope of the invention, but rather as particular embodiments representative of the invention.

## EXAMPLE 1

An aqueous solution having a 40% by weight concentration of volatile corrosion inhibitor materials was prepared by dissolving the following corrosion inhibitor mixture in water:

| Corrosion Inhibitor Component | Concentration (Weight) |
|-------------------------------|------------------------|
| Cyclohexyl-ammonium Benzoate  | 50%                    |
| Ammonium Benzoate             | 25%                    |
| Sodium Benztiazole            | 5%                     |
| Monoethanolammonium Benzoate  | 10%                    |
| Imidazoline Nitrate           | 10%                    |

Open cell foam having a density of about 1.1 to 1.2 pounds per cubic foot is available from Future Foam, Inc. of Council Bluffs, Iowa in sheet form with a thickness of 0.25 inch. An open cell foam roll was immersed in the corrosion inhibitor solution in a roll coating apparatus having a feed speed of 20 ft/min, and was subsequently air dried for 10 minutes at 175° F. The resultant product contained about 60% by weight volatile corrosion inhibitor materials.

## EXAMPLE 2

An open cell foam from Future Foam, Inc. having a density of about 1.35 to 1.5 pounds per cubic foot and a thickness of 0.25 inches was immersed in the corrosion inhibitor solution of Example 1 and subsequently dried. The resultant product contained about 35% by weight volatile corrosion inhibitor materials.

## EXAMPLE 3

An aqueous solution was prepared containing 40% by weight of volatile corrosion inhibitor materials in the following ratios:

| Corrosion Inhibitor Component | Concentration (Weight) |
|-------------------------------|------------------------|
| Cyclohexyl-ammonium Benzoate  | 70%                    |
| Benzotiazole                  | 30%                    |

The open cell foam material of Example 1 was immersed in the above aqueous solution in the roll coating apparatus and subsequently dried as described above. The resultant product contained about 60% by weight volatile corrosion inhibitor material, and is particularly useful in the corrosion protection of copper and aluminum.

## DISCUSSION

The volatile corrosion inhibitor loaded foam was cut to a desired size and enclosed in the inner enclosure barrier as a vapor phase corrosion inhibitor-emitting substrate. The inner enclosure barrier was formed of two sheets of Tyvek® 1059 material available from E.I. du Pont de Nemours & Company, with each sheet having a caliper thickness of 125-175 µm. The respective perimeter portions of each sheet are heat-sealed to one another in a conventional heat-sealing apparatus operating at 110° C.

The combination of the substrate within the inner enclosure barrier was disposed within the outer enclosure barrier that is formed of two sheets of metallized film available from LPS Industries of Moonachie, N.J. under the designation VF42. The metallized film layers were sealed to one another at their respective perimeters through an impulse heat sealing process at the following operating conditions:

Temperature=350° F.  
Pressure=26 psi  
Time=0.75 sec

The seal between the two film layers of the outer enclosure barrier is preferably gas-tight so as to render the entire boundary gas-impermeable.

15 The effectiveness of the loaded substrates as packaged within the enclosure barriers as described above was analyzed using Time of Flight Surface Ion Mass Spectroscopy (TOF-SIMS) on copper wafers within a lot box placed between about 0.1 and up to 30 cm from the vapor phase corrosion inhibitor-emitting substrates. In addition, the analysis reviewed the extent to which the corrosion protection characteristic was retained on the respective corrosion-susceptible wafers. Additional testing over a temperature range from 20 -20° C. to +250° C. of a fully treated wafer showed significant desorption beginning at 150° C. The long-term retention of the corrosion inhibition characteristic at ambient conditions is important in applications such as within the semiconductor industry, as corrosion-susceptible wafers may experience varying degrees of moisture and airborne chemical 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630

-continued

| Sample Conditions                                                                                                                                                                                                                                                                                                      | Maximum Vapor Phase Corrosion Inhibitor Concentration (PPB) |
|------------------------------------------------------------------------------------------------------------------------------------------------------------------------------------------------------------------------------------------------------------------------------------------------------------------------|-------------------------------------------------------------|
| gas-impermeable outer enclosure but still disposed within a gas-permeable, solid particle-impermeable material enclosure and exposed to the ambient environment in this condition for 6 months prior to testing in empty lot box.                                                                                      |                                                             |
| 6 1 VCI-containing substrate in accordance with Example 1, opened from an outer gas-impermeable outer enclosure but still disposed within a gas-permeable, solid particle-impermeable material enclosure and exposed to the ambient environment in this condition for about 1 month prior to testing in empty lot box. | 38                                                          |
| 7 1 VCI-containing substrate in accordance with Example 1, opened from an outer gas-impermeable outer enclosure but still disposed within a gas-permeable, solid particle-impermeable material inner enclosure, and tested immediately in an empty lot box.                                                            | 53                                                          |

The invention has been described herein in considerable detail in order to comply with the patent statutes, and to provide those skilled in the art with the information needed to apply the novel principles and to construct and use embodiments of the invention as required. However, it is to be understood that the invention can be carried out by specifically different devices and that various modifications can be accomplished without departing from the scope of the invention itself.

What is claimed is:

1. A method for inhibiting corrosion of corrosion-susceptible material, said method comprising:
  - (a) providing a corrosion inhibitor package having:
    - (i) a first enclosure barrier comprising one or more gas-impermeable materials and defining a first enclosed space;
    - (ii) a second enclosure barrier comprising a gas-permeable, solid particle-impermeable material, said second enclosure barrier being disposed in said first enclosed space and defining a second enclosed space inside of said first enclosed space, said second enclosure barrier having mono-direction emissivity and permitting vapors to pass through said second enclosure barrier from within the second enclosed space; and
    - (iii) a substrate having one or more volatile corrosion inhibitor materials disposed thereon, said substrate being disposed within said second enclosed space;
  - (b) breaching said first enclosure barrier to thereby render said second enclosed space in gas communication with ambient environment external to said corrosion inhibitor package; and
  - (c) placing said corrosion inhibitor package in proximity to corrosion-susceptible material.
2. A method as in claim 1 wherein the breaching includes removing at least a portion of said first enclosure barrier from said corrosion inhibitor package.
3. A method as in claim 1 wherein said corrosion-susceptible material is metal surfaces of a semiconductor device.
4. A method as in claim 1 wherein said corrosion-susceptible material is metal surfaces of a semiconductor wafer.

5. A method as in claim 1 wherein said corrosion inhibitor package is placed between about 0.1 and 30 cm from said corrosion-susceptible material.
6. A method as in claim 1, including substantially immediately placing said corrosion inhibitor package in proximity to said corrosion-susceptible material upon breach of said first enclosure barrier.
7. A method as in claim 1, wherein said substrate includes an open cell foam divided into a plurality of distinct foam pieces having a mean diameter of between about 0.25 mm and 0.5 mm.
8. A method as in claim 1, wherein said one or more volatile corrosion inhibitor materials are disposed on said substrate with a loading of 35 wt % to 60 wt %.
9. A method as in claim 1, wherein said one or more gas-impermeable materials include a metalized polyethylene terephthalate film including a vapor deposited film of metal.
10. A method as in claim 1, wherein said one or more gas-impermeable materials of said first enclosure barrier include a self-supporting gas-impermeable material defining an annular flange.
11. A method as in claim 10, wherein said one or more gas-impermeable materials of said first enclosure barrier further include a barrier layer secured to the annular flange.
12. A method for inhibiting corrosion of corrosion-susceptible material, said method comprising:
  - (a) providing a corrosion inhibitor package having:
    - (i) a first enclosure comprising one or more gas-impermeable materials and defining a first enclosed space;
    - (ii) a second enclosure defining a second enclosed space within the first enclosed space, the second enclosure having mono-direction emissivity and permitting vapor to pass through the second enclosure from the inside of the second enclosed space; and
    - (iii) a substrate having one or more volatile corrosion inhibitor materials disposed thereon, said substrate being disposed within said first enclosed space;
  - (b) breaching said enclosure barrier to thereby render said substrate in gas communication with ambient environment external to said enclosure barrier; and
  - (c) placing said substrate in proximity to said corrosion-susceptible material.
13. A method as in claim 12 wherein the breaching includes removing at least a portion of said enclosure barrier from said corrosion inhibitor package.
14. A method as in claim 12 wherein said corrosion-susceptible material is metal surfaces of a semiconductor device.
15. A method as in claim 12 wherein said corrosion-susceptible material is metal surfaces of a semiconductor wafer.
16. A method as in claim 12 wherein said substrate is placed between about 0.5 and 30 cm from said corrosion-susceptible material.
17. A method as in claim 12, including substantially immediately placing said substrate in proximity to said corrosion-susceptible material upon breach of said enclosure barrier.
18. A method as in claim 12, wherein said substrate includes an open cell foam divided into a plurality of distinct foam pieces having a mean diameter of between about 0.25 mm and 0.5 mm.
19. A method as in claim 12, wherein said one or more volatile corrosion inhibitor materials are disposed on said substrate with a loading of 35 wt % to 60 wt %.
20. A method as in claim 12, wherein said one or more gas-impermeable materials include a metalized polyethylene terephthalate film including a vapor deposited film of metal.

**11**

**21.** A method as in claim **12**, wherein said one or more gas-impermeable materials of said first enclosure include a self-supporting gas-impermeable material defining an annular flange.

**22.** A method as in claim **21**, wherein said one or more of said gas-impermeable materials first enclosure further include a barrier layer secured to the annular flange.

**23.** A method for inhibiting corrosion of corrosion-susceptible material, said method comprising:

(a) providing a corrosion inhibitor package having:

- (i) a first enclosure barrier defining a first enclosed space and comprising a gas-impermeable material including a metalized polyethylene terephthalate film including vapor deposited metal;
- (ii) a second enclosure barrier disposed within the first enclosed space and defining a second enclosed space, the second enclosure barrier being mono-direction emissive and permitting vapors to pass through said second enclosure barrier from within the second enclosed space; and

5

(iii) a substrate having one or more volatile corrosion inhibitor materials disposed thereon, said substrate being disposed within said second enclosed space;

(b) breaching said first enclosure barrier to thereby render said second enclosed space in gas communication with ambient environment external to said corrosion inhibitor package; and

(c) placing said corrosion inhibitor package in proximity to corrosion-susceptible material.

**10** **24.** A method as in claim **23**, wherein the first enclosure barrier further comprises a self-supporting barrier material defining an annular flange, the metalized polyethylene terephthalate film secured to the annular flange.

**15** **25.** A method as in claim **23**, wherein said substrate includes an open cell foam divided into a plurality of distinct foam pieces having a mean diameter of between about 0.25 mm and 0.5 mm.

**20** **26.** A method as in claim **23**, wherein said one or more volatile corrosion inhibitor materials are disposed on said substrate with a loading of 35 wt % to 60 wt %.

\* \* \* \* \*